

## UNITED STATES PATENT OFFICE.

HANS RATHSBURG, OF FURTH, GERMANY.

## PRIMING COMPOSITION AND PROCESS FOR PRODUCING THE SAME.

No Drawing.

Application filed October 19, 1921. Serial No. 508,826.

*To all whom it may concern:*

Be it known that I, HANS RATHSBURG, a citizen of Germany, residing at Furth, Bavaria, Republic of Germany, have invented 5 new and useful Improved Priming Compositions and Processes for Producing the Same, of which the following is a specification.

My invention relates to an improved 10 priming composition and its object is to produce a standard priming composition by replacing the fulminate of mercury by a more suitable substance.

With this end in view it was proposed to 15 mechanically add suitable bodies or explosives. For instance so-called ignition or flame transmitters were pressed upon the leadazid, which is inflammable with difficulty only, for example a mixture of rhodan lead and 20 potassium chlorate and also di- or trinitro-resorcinate of lead or potassium dinitro-dinitrosobenzole, while these and similar substances in order to charge percussion-caps and Flobert ammunition were mixed with 25 the fulminate of mercury or the leadazid. Such processes have already become known, although only very recently.

It has now been ascertained that the lead salt of the trinitro-phloroglucine comes very 30 much nearer the object aimed at of obtaining a standard priming composition. In contradistinction to the mercury fulminate of this salt may be stored for any length of time, even in heated, damp rooms. A fur- 35 ther advantage of this salt over the mercury fulminate and recently employed or proposed primings is its total indifference to metals in humid air, more particularly to

aluminiun, brass and copper and also to carbonic acid and other obnoxious gases, as they 40 occur, for instance, in coal mines.

When subjected to heat, it is also far superior to the fulminate of mercury, inasmuch as it only evaporates at a 60-70° higher 45 temperature than the latter. Its solubility is also considerably less than that of the fulminate of mercury. It is, furthermore, far easier inflammable than the leadazid and it excels the fulminate of mercury also as a 50 transmitter of flames or sparks.

These advantages clearly show that a considerable technical progress is attained by employing these salts as primings in the manufacture of ammunition.

It has also been found that the lead trinitrophloroglucinate, which on ignition generates a stronger gas-pressure than mercury fulminate, may easily be phlegmatized or quickened in its action as desired or required, by mixing it mechanically with milder or more 55 powerful explosives.

What I claim as my invention and desire to secure by United States Letters Patent is:

The improved process for the production 65 of a priming composition, which comprises employing the lead salt of the trinitrophloroglucine.

In testimony whereof I have signed my name to this specification in the presence of 70 two subscribing witnesses.

DR. ING. HANS RATHSBURG.

Witnesses:

Dr. EMIL BURKARD,  
KARL WEISS.